

## UNITED STATES PATENT OFFICE.

FRANCIS I. DU PONT AND ERNEST DU PONT, OF WILMINGTON, DELAWARE, ASSIGNEES  
TO U. S. F. POWDER COMPANY, OF WILMINGTON, DELAWARE, A CORPORATION OF  
DELAWARE.

## FLASHLESS CANNON POWDER.

No Drawing.

Application filed November 13, 1926. Serial No. 148,313.

This invention relates to flashless cannon powders; and it comprises a smokeless and flashless powder of the usual grain shapes employed in ordnance, each grain being composed of an integral body of colloided nitrocellulose containing distributed therethrough isolated particles of a mixture of charcoal with a nitrate, usually potassium nitrate, the proportions of charcoal and of nitrate frequently being about equal; all as more fully hereinafter set forth and as claimed.

Smokeless powder for cannons is made of colloided nitrocellulose. Sometimes nitro-glycerin is present, as in the English cordite. The particular solvent used in colloidizing is important as regards the character of the powder and its ballastic properties. Ether-alcohol and acetone are solvents commonly used. For large guns the colloided powder is generally cut into sticks carrying longitudinal perforations. These perforations are to give a progressively increasing burning area.

All smokeless ordnance powders have the defect of giving a muzzle flash; a flame of secondary combustion beyond the muzzle as the hot explosion products meet the air. For military purposes this flash is seriously detrimental. In various prior and copending applications we have described and claimed flashless smokeless propellant powders and methods of making the same. In explosive units made according to these inventions an integral body of colloided powder contains uniformly distributed particles of what we have termed a "flame propagating agent"; the body of colloided nitrocellulose is a sort of honeycomb with the agent in the cells. The office of the agent is to provide new burning areas as combustion reaches the cells. Another type of progressive increase of burning area is superimposed upon that afforded by the usual perforations which are here also used. As flame propagating agents we have disclosed a variety of materials including ammonium nitrate, barium nitrate, potassium bichromate, etc. In one of said applications, filed April 24, 1920, as Serial No. 376,267, we have described and claimed a type of flashless powder wherein flashlessness is secured by a thorough distribution of fine grained black powder through the granule; the

black powder existing as isolated grains in the cells of what may be termed a honeycomb of colloided nitrocellulose. This black powder is of the usual composition; a relatively large amount of potassium nitrate with less amounts of sulfur and charcoal.

We have found that in some relations a proportion of nitrate to charcoal less than that existing in black powder is better; and that in some of these relations it is desirable that a mixture of charcoal and nitrate only be used; that sulfur shall be absent.

Sulfur is always a component of black powder. The absence of sulfur is particularly desirable where the colloided body contains nitroglycerin. While various other proportions of charcoal and potassium nitrate may be employed, we have found that in most instances a mixture of about equal parts is best. Instead of potassium nitrate we may use barium nitrate or even sodium or ammonium nitrate but we find potassium nitrate on the whole the best nitrate to use.

In a practical embodiment of the present invention, equal parts of potassium nitrate and charcoal may be worked together into a fine grain composition in much the way used in making black powder except that no sulfur is added. The product is advantageously of about the same fineness as ordinary meal powder. In making a typical flashless powder under the present invention about five parts of this product is placed in a standard black powder wheel mill with 100 parts of pulped nitrocellulose. The materials are incorporated together until an even distribution of the charcoal-nitrate composition is effected. A blending liquid may be used to aid in this incorporation. This blending liquid may be a non-solvent for nitrocellulose, such as for instance gasoline, as described in the copending application Serial No. 376,267 referred to above, or the blending liquid may be one useful in colloidizing, such as alcohol or ether or a mixture of the two. After the incorporation is complete the mixture is colloided in any of the usual ways so as to obtain an integral mass of nitrocellulose; this mass containing the charcoal-nitrate grains uniformly distributed therethrough. This colloided body may be formed into usual types of grain by the usual methods and with the use of the ordinary types of apparatus. Ordinarily it

finally goes through die presses to furnish longitudinal strings or cords having the seven longitudinal perforations usual in units or grains for ordnance purposes.

5 Any of the varieties of charcoal used in making powder may be here employed. Carbon from other sources, such as gas black, may be used in lieu of charcoal.

What we claim is:—

10 1. As a flashless powder, colloided nitro-cellulose containing distributed grains of a mixture composed of charcoal and a nitrate and free of sulfur.

15 2. As a flashless powder, colloided nitro-cellulose containing distributed grains of a mixture composed of charcoal and potassium nitrate and free of sulfur.

3. As a flashless powder, colloided nitro-cellulose containing distributed grains of a

mixture composed of charcoal and a nitrate, 20 the nitrate and the charcoal being present in about equal amounts.

4. As a flashless powder, colloided nitro-cellulose containing nitroglycerin and also containing distributed grains of a mixture 25 composed of charcoal and a nitrate.

5. As a flashless powder, colloided nitro-cellulose containing nitroglycerin, colloiding being effected with a solvent comprising acetone, said colloided nitrocellulose containing distributed grains of a mixture composed of charcoal and a nitrate.

In testimony whereof, we have hereunto affixed our signatures at Wilmington, Delaware, this 12th day of November, 1926.

FRANCIS I. DU PONT.  
ERNEST DU PONT.